

# United States Patent Office

2,981,623

Patented Apr. 25, 1961

1

2,981,623

## PHOTOGRAPHIC DEVELOPERS

Lothar Burgardt, Leverkusen-Bayerwerk, Willibald Pelz, Köln-Stammheim, Ottmar Wahl, Opladen, and Heinz Sassemann, Burscheid, Germany, assignors to Agfa Aktiengesellschaft, Leverkusen, Germany, a corporation of Germany

No Drawing. Filed Mar. 14, 1955, Ser. No. 494,221

Claims priority, application Germany Mar. 15, 1954

11 Claims. (Cl. 96—60)

The present invention relates to photographic developer substances and more especially to substances derived from 4-amino-pyrazolones-(5).

As photographic developers, it has been the practice hitherto generally to employ substances which belong to the class of aromatic polyvalent hydroxy compounds, amino-hydroxy compounds or polyvalent amino compounds. Compounds of the heterocyclic class are known to have developer properties (German Patent No. 646,516), inter alia, 5-pyrazolones, substituted in the 4-position with an amino group, which 5-pyrazolones contain the  $\alpha$ -aminoketone structure in the heterocyclic nucleus. These aminopyrazolones are, however, exclusively substances which are alkylated in the 3-position. These compounds have not been used in practice as developers, since they are quite unstable with relatively small intensity of development and show a strong tendency to fogging.

It has now been found that 4-aminopyrazolones of the following constitution do not have these properties which are disadvantageous for use in practice as developers:



wherein  $R_1$  may represent  $-\text{OH}$ ,  $-\text{O-alkyl}$ ,  $-\text{O-aryl}$ ,  $-\text{O-aralkyl}$ ,  $\text{NH}_2$  or substituted  $\text{NH}_2$  groups,  $-\text{NH}-\text{NH}_2$  or substituted hydrazide groups,  $-\text{NH}-\text{OH}$  or an azide group and also alkyl, aryl or aralkyl radicals.  $R_2$  may represent hydrogen, alkyl, aralkyl, aryl groups or substituted aryl groups or heterocyclic radicals.

It has surprisingly been found that such compounds represent excellent photographic developer substances, since they operate without fogging with a surprisingly high development intensity and are sufficiently stable in order to be used practically as developers. The developer substances may either be used independently or with advantage in combination with known developer substances, whereby they either work more quickly owing to their great rapidity, i.e. develop images to the same gamma value in a shorter time, or they develop a specific photographic material to higher gamma values with the same development period. Moreover, the property of super-additivity may also frequently be used with advantage in combination with other developer substances for producing higher sensitivity. Suitable known developing substances are for instance polyhydric phenols such as pyrocatechol, hydroquinone, pyrogallol, o- and p-aminophenols such as p-methyl-aminophenol, N-p-oxyphenylglycin, o- and p-phenylenediamines. These substances may be substituted in the amino group or in the aromatic nucleus. The developer substances are suitable for the development of the widest possible variety of silver halide emulsions, for highly sensitive negative emul-

2

sions and also for less sensitive positive emulsions or paper emulsions. The developer substances are suitable both for direct development of silver halide layers and for the production of photographic reversal images. Yet another advantage of the said compounds, as compared with the known developer substances, is their water-solubility and alkali-solubility, which is sometimes high and renders it possible for strongly concentrated developer solutions to be manufactured and brought on to the market. The developer substances according to the present invention may be incorporated into silver halide emulsion layers which are developed by alkaline solution containing, if desired, developer substances.

Examples of the aforementioned pyrazolones are:

- Examples of the aforementioned pyrazolones are:  
15 4-amino-5-pyrazolones-3-carboxylic acid ethyl ester, 1-phenyl-4-amino-5-pyrazolones-3-carboxylic acid ethyl ester, 1-phenyl-4-amino-5-pyrazolone-3-carboxylic acid amide, 1 - (p - ethoxy - phenyl) - 4 - amino - 5 - pyrazolone-3-carboxylic acid ethyl ester, 1-phenyl-3-(methane  
20 sulphohydrazo-carbonyl)-4-amino-5-pyrazolone or 1-(p-sulphophenyl) - 4 - amino - 5 - pyrazolone - 3 - carboxylic acid methyl ester. A large number of further compounds are possible, according to substitution of the radicals  $R_1$  and  $R_2$ . The production of these aminopyrazolones is  
25 carried out according to known processes. For example, suitable pyrazolones may be transformed by treatment with nitrite into the isonitroso-compounds and the latter by reduction with tin into the associated amino compounds. The reduction of the isonitroso-compounds  
30 may also be carried out according to other known processes, for example with zinc and glacial acetic acid or catalytically. Another available method for the production of such compounds is based upon the reductive splitting of azo dyestuffs, which are obtained by coupling  
35 suitable pyrazolones with diazonium salts.

### EXAMPLE 1

For developing a commercially available black-and-white film with the sensitivity of 17/10 DIN, there is employed the following developer solution:

|                                                                            |    |      |
|----------------------------------------------------------------------------|----|------|
| Sodium sulphite anhydrous                                                  | g  | 80   |
| Hydroquinone                                                               | g  | 3    |
| Borax                                                                      | g  | 3    |
| 45 KBr                                                                     | g  | 0.5  |
| 1-phenyl-4-amino-5-pyrazolone - 3 - carboxylic acid<br>amide hydrochloride | g  | 2.5  |
| Water                                                                      | cc | 1000 |

50 The developer solution has a soft action and is fine-grained with high speed. With a development period of nine minutes, the film shows a fogging of 0.08. The development period for a like film material (17/10 DIN) in a corresponding metol-hydroquinone developer, which 55 contains 1.7 g. of metol (=molar quantity) instead of the 1-phenol-4-amino-5-pyrazolone-3-carboxylic acid amide hydrochloride, is eighteen minutes for producing similar sensitivity and gradation. (Fogging 0.17.)

60 The following table, in which the gamma values and fogging values are entered in dependence upon the development period, illustrates the great rapidity and contrast of the photographic developer, the figures in brackets representing the values for like material treated in a corresponding metol-hydroquinone developer:

|    |     | Development period (minutes) | Gamma value | Fogging     |
|----|-----|------------------------------|-------------|-------------|
| 70 | 4½  |                              | 0.3 (0.25)  | 0.04 (0.04) |
|    | 9   |                              | 0.49 (0.3)  | 0.08 (0.05) |
|    | 13½ |                              | 0.64 (0.44) | 0.13 (0.09) |
|    | 18  |                              | 0.7 (0.5)   | 0.13 (0.17) |

## 3

1-phenyl-4-amino-pyrazolone-3-carboxylic acid amide is prepared as follows:

206 g. of 1-phenyl-pyrazolone-3-carboxylic acid ethyl ester are heated in the autoclave with

380 g. of ammonia (25%) to 80-85° C. for 6 hours, a part of the ammonia is distilled off and the content dissolved in

500 cc. of water. After addition of

56 g. of nitrite, the solution is slowly introduced with stirring at 0° C. into

1000 cc. of hydrochloric acid (10%), filtered with suction and the filtered substance washed with hydrochloric acid (10%) and methanol.

Yield: 235 g. of isonitroso derivative.

50 g. of the isonitroso product are dissolved in

500 cc. of glacial acetic acid and treated at 40-50° C. with zinc dust until decolorization. After filtering the solution and passing in hydrogen chloride, the hydrochloride of the aminopyrazolone is obtained in good yield; it is filtered with suction, the filtered substance dissolved in little water while hot, precipitated with hydrochloric acid and dried in vacuum over caustic potash after filtering with suction.

Yield: 40 g.

## EXAMPLE 2

For developing a commercially available black-and-white film with the sensitivity of 17/10 DIN, there is employed the following developer solution:

|                                                                                          |    |      |
|------------------------------------------------------------------------------------------|----|------|
| Anhydrous sodium sulphite                                                                | g  | 80   |
| Borax                                                                                    | g  | 3    |
| KBr                                                                                      | g  | 0.5  |
| Metol                                                                                    | g  | 1.5  |
| Methane-sulphohydrazide of 1-phenyl-4-amino-5-pyrazolone-3-carboxylic acid hydrochloride | g  | 9.5  |
| Water                                                                                    | cc | 1000 |

Strongly-acting fine-grain developer. (Development period: eight to nine minutes.)

For comparison purposes, similar film material (17/10 DIN) is developed after exposure in the sensitometer in the corresponding metol-hydroquinone developer (containing the molar amount of hydroquinone, namely 3 g., instead of the aminopyrazolone) and the gamma values and also development fogging are measured after different development periods and compared with correspondingly treated photographic material which is developed in the developer of Example 2, the figures in brackets representing gamma values and fogging values of the film material developed in the corresponding metol-hydroquinone developer.

| Development period (minutes) | Gamma value | Fogging     |
|------------------------------|-------------|-------------|
| 4½                           | 0.5 (0.25)  | 0.07 (0.04) |
| 9                            | 0.75 (0.3)  | 0.10 (0.07) |
| 13½                          | 0.9 (0.43)  | 0.10 (0.09) |
| 18                           | 1.0 (0.46)  | 0.12 (0.11) |

The methane sulphohydrazide of 1-phenyl-4-amino-5-pyrazolone-3-carboxylic acid is prepared as follows:

206 g. of 1-phenyl-pyrazolone-3-carboxylic acid ethylester are introduced into

120 cc. of alcohol and heated to boiling temperature for 5 hours with

120 cc. of hydrazinehydrate (83%) while stirring under reflux. After cooling the reaction mixture is introduced with stirring into

200 cc. of hydrochloric acid (20%) and 200 g. of ice, filtered with suction, the filtered substance washed with water and dried.

Yield: 220 g. of hydrazide; M.P.: 252-254° C.

220 g. of the hydrazide are dissolved in

## 4

430 cc. of sodium hydroxide solution (5%) and reacted dropwise at 10-15° C. with

125 g. of methane sulphonylchloride with the simultaneous addition of sodium hydroxide solution (10%) at such a rate that the solution is kept alkaline against phenolphthalein. The solution is stirred for a further 30 minutes and precipitation effected with hydrochloric acid (10%) after filtering, then filtered with suction and the filtered substance washed. The wet filter cake is dissolved in sodium hydroxide solution (10%), mixed with

70 g. of nitrite and introduced with stirring into

300 cc. of hydrochloric acid and

700 g. of ice. The isonitroso product obtained is filtered with suction, the filtered substance stirred with water, filtered with suction and dried.

Yield: 250 g.

The isonitroso compound can be reduced with tin sponge and hydrochloric acid according to the process described in Arch. Pharm., 278 (1940), p. 330.

## EXAMPLE 3

|                                                                  |    |      |
|------------------------------------------------------------------|----|------|
| Anhydrous sodium sulphite                                        | g  | 125  |
| Soda                                                             | g  | 12   |
| KBr                                                              | g  | 1.5  |
| 4-amino-5-pyrazolone-3-carboxylic acid ethyl ester hydrochloride | g  | 13   |
| Water                                                            | cc | 1000 |

The developer develops negatives brilliantly with fine-grain and free from fogging. (Development period: eight minutes.)

4-amino-5-pyrazolone-3-carboxylic acid ethyl ester is prepared as follows:

150 g. of sodium acetate, 790 g. of sodium oxalate and 630 g. of hydrazine sulfate in

40 3000 cc. of water are heated to boiling temperature with stirring for 6 hours and then stirred in the cold. The pyrazolone formed is separated by filtering with suction, washed with water, stirred twice with 100 cc. of methanol each and filtered with suction.

Yield: 430 g.

430 g. of the pyrazolone are dissolved in

1000 cc. of hydrochloric acid (1:1) at 50° C., the undissolved portion is separated by filtering and the solution is mixed at 10-15° C. with

50 170 g. of nitrite in 300 cc. of water. After filtering with suction, washing water and drying

380 g. of isonitroso derivative are obtained. The derivative is mixed with

55 100 cc. of alcohol, reacted while stirring with 1000 cc. of hydrochloric acid and reduced by gradual addition of 250 g. of tin sponge within 5 hours. The hydrochloride is filtered with suction, dissolved in 1000 cc. of hot water, filtered and precipitated in the cold with

150 cc. of hydrochloric acid. After filtering with suction, washing with little water and drying in vacuum.

340 g. of the developer substance are obtained.

## EXAMPLE 4

|                                                                                      |    |      |
|--------------------------------------------------------------------------------------|----|------|
| Anhydrous sodium sulphite                                                            | g  | 40   |
| Potash                                                                               | g  | 40   |
| KBr                                                                                  | g  | 2    |
| Hydroquinone                                                                         | g  | 6    |
| 70 1 - phenyl - 4 - amino - 5 - pyrazolone - 3 - carboxylic acid amide hydrochloride | g  | 10   |
| Water                                                                                | cc | 1000 |

Very powerful negative developer. (Development period: three minutes.)

## EXAMPLE 5

## Solution A

|                                                                         |   |      |
|-------------------------------------------------------------------------|---|------|
| Water                                                                   | g | 1000 |
| 1-phenyl-4-amino-5-pyrazolone-3-carboxylic acid hydrazide hydrochloride | g | 60   |
| Potassium metabisulphite                                                | g | 20   |
| KBr                                                                     | g | 25   |

## Solution B

|                |    |      |
|----------------|----|------|
| Water          | cc | 1000 |
| Caustic potash | g  | 50   |

Soft high-speed developer for negatives. (Development period: forty seconds.)

1-phenyl-4-amino-5-pyrazolone-3-carboxylic acid hydrazide can be prepared as follows:

1-phenyl-5-pyrazolone-3-carboxylic acid ethyl ester is converted to the isonitroso compound according to Arch. Pharm., 278 (1940), p. 330.

130 g. of the isonitroso compound are stirred at room temperature for 6 hours with 130 g. of hydrazine hydrate (78%), reacted with methanol and filtered with suction.

The reaction product is reduced with tin sponge and hydrochloric acid according to Arch. Pharm., 278 (1940), p. 330.

## EXAMPLE 6

|                                                                                         |    |      |
|-----------------------------------------------------------------------------------------|----|------|
| Metol                                                                                   | g  | 1    |
| Sodium sulphite anhydrous                                                               | g  | 13   |
| Soda                                                                                    | g  | 26   |
| KBr                                                                                     | g  | 1    |
| 1 - phenyl - 4 - amino - 5 - pyrazolone - 3 - carboxylic acid ethyl ester hydrochloride | g  | 8    |
| Water                                                                                   | cc | 1000 |

Normal developer for silver bromide and silver chloride papers.

This aminopyrazolone is produced according to Arch. Pharm., 278 (1940), p. 330.

## EXAMPLE 7

In the developer of Example 3, the hydrochloride of 4-amino-5-pyrazolone-3-carboxylic acid ester is replaced by 15 g. of 1-(p'-sulfonylphenyl)-4-amino-5-pyrazolone-3-carboxylic acid ethyl ester. The developer is of high stability and develops negatives brilliantly and free from fogging.

1 - (p' - sulfophenyl) - 4 - amino - 5 - pyrazolone - 3 - carboxylic acid ethyl ester is prepared as follows:

31.2 g. of 1-(p'-sulfonylphenyl)-5-pyrazolone-3-carboxylic acid ethyl ester are dissolved in 150 cc. of sodium hydroxide solution (10%), mixed with 7.0 g. of nitrite dissolved in little water, and introduced dropwise with stirring at 5-10° C. into hydrochloric acid. The isonitroso product precipitating in yellow flocs is filtered with suction, the filtered substance stirred with hot alcohol and dried by suction filtering.

34 g. of the nitroso compound are mixed with stirring with 20 cc. of alcohol and 120 cc. of hydrochloric acid and reduced with 24 g. of tin sponge as usual. The aminopyrazolone is filtered with suction and recrystallized from water.

## EXAMPLE 8

|                                                                                |    |            |
|--------------------------------------------------------------------------------|----|------------|
| Metol                                                                          | g  | 0.75       |
| Hydroquinone                                                                   | g  | 2          |
| 1 - phenyl-4-amino-5-pyrazolone-3-carboxylic acid-(ethanolamide)-hydrochloride | g  | 1.5        |
| Sodium sulfite anhydrous                                                       | g  | 80         |
| Borax                                                                          | g  | 3          |
| Potassium bromide                                                              | g  | 0.5        |
| Water                                                                          | cc | Up to 1000 |

High-speed fine-grain developer; development period: 8 minutes.

1-phenyl-4-amino-5-pyrazolone-3-carboxylic acid-(ethanolamide) is prepared as follows:

5 20.6 g. of 1-phenyl-5-pyrazolone-3-carboxylic acid ethyl ester and 20 cc. of ethanol amine (50%) are heated under reflux to 140° C. for 5 hours, diluted with water and introduced with stirring into hydrochloric acid (10%). The reaction product is filtered with suction and the filtered substance recrystallized from methanol (50%).

Yield: 28 g. (wet).

The ethanol amide is dissolved in sodium hydroxide solution (3%), mixed with 8 g. of nitrite, introduced with stirring into hydrochloric acid (10%), filtered with suction and recrystallized from alcohol.

Yield: 23.5 g.

20 23.5 g. of the isonitroso product are dissolved in 150 cc. of methanol, mixed with

1 g. of Raney nickel and stirred at 60-70° C. in the autoclave until hydrogen absorption is complete. The hydrogenation solution is filtered with suction in the heat and precipitated with hydrochloric acid.

Yield: 18 g.

## EXAMPLE 9

|                                                                                                   |    |            |
|---------------------------------------------------------------------------------------------------|----|------------|
| 1 - (p'-aminophenyl) - 4 - amino - 5 - pyrazolone - 3 - carboxylic acid ethyl ester hydrochloride | g  | 3          |
| Sodium sulfite anhydrous                                                                          | g  | 40         |
| Hydroquinone                                                                                      | g  | 6          |
| Soda                                                                                              | g  | 20         |
| Potassium bromide                                                                                 | g  | 1          |
| Water                                                                                             | cc | Up to 1000 |

Soft-acting negative developer for orthochromatic and panchromatic photographic materials; development period: 5 minutes.

40 1-(p'-aminophenyl) - 4 - amino - 5 - pyrazolone - 3 - carboxylic acid ethyl ester is prepared as follows:

27.7 g. 1-(p'-nitrophenyl)-5-pyrazolone-3-carboxylic acid ethyl ester are dissolved in

45 150 cc. of sodium hydroxide solution (3%), reacted with 7.5 g. of nitrite and introduced with stirring into 100 cc. of hydrochloric acid and

100 g. of ice. The isonitroso product formed is filtered with suction, washed with water and dried.

30.5 g. of the isonitroso product are suspended with

50 50 cc. of alcohol and

200 cc. of hydrochloric acid and treated in the usual manner with

60 60 g. of tin sponge until decolorization. Apart from the nitro group, the nitro grouping is also completely reduced. The diamine is filtered with suction, dissolved in little water in the heat and precipitated with hydrochloric acid while cooling. The hydrochloride is filtered with suction and dried in vacuum over caustic potash.

## EXAMPLE 10

In the developer of Example 4, the hydrochloride of 1-phenyl-4-amino-5-pyrazolone-3-carboxylic acid ester is replaced by 10 g. of 1-(p'-ethoxyphenyl)-4-amino-5-pyrazolone-3-carboxylic acid. A negative developer is thus obtained.

Development periods: 3-4 minutes.

1-(p'-ethoxyphenyl) - 4 - amino - 5 - pyrazolone - 3 - carboxylic acid is prepared as follows:

70 20 g. p-ethoxyphenylhydrazine-hydrochloride are introduced into

100 cc. of alcohol,

10 g. of sodium acetate are added and reacted at room temperature dropwise with

75 20 g. of oxalate. After stirring for one hour the mixture

is filtered with suction and the filtered substance recrystallized from alcohol. 1-(p'-ethoxyphenyl)-5-pyrazolone-3-carboxylic acid is obtained by stirring the ester in 2 N sodium hydroxide solution for some hours and isolated by acidifying the alkaline solution.

16 g. of the carboxylic acid are dissolved in 70 cc. of sodium hydroxide solution (4%), mixed with 4.5 g. of nitrite and introduced with stirring into 100 cc. of hydrochloric acid (1:1). The isonitroso product formed is filtered with suction, the filtered substance washed with water and dried. The reduction is effected with tin sponge and hydrochloric acid in the usual manner.

## EXAMPLE 11

1 - (2'-tetrahydrothiophenesulfone)-4-amino-5-pyrazolone-3-carboxylic acid ethyl ester hydrochloride

|                          |                 |
|--------------------------|-----------------|
| g--                      | 14              |
| Sodium sulfite anhydrous | g-- 125         |
| Soda                     | g-- 6           |
| Potassium bromide        | g-- 2.5         |
| Water                    | cc-- Up to 1000 |

Very soft fine-grain developer; development period: 12-14 minutes.

1 - (2' - tetrahydrothiophenesulfone) - 4 - amino - 5 - pyrazolone-3-carboxylic acid ethyl ester is prepared as follows:

31.5 g. of an aqueous hydrazine solution (35%) are reacted with 16.0 g. of butadiene sulfone, kept at 75° C. for 30 hours and the major quantity of water removed in vacuum. 15 g. of the resulting hydrazine are heated to 45° C. for 5 hours with 21 g. of sodium oxalate, 50 cc. of alcohol (50%) and 6.6 cc. of glacial acetic acid. The alcohol is distilled off in vacuum, the residue suspended with dilute hydrochloric acid, filtered with suction and the filtered substance recrystallized from acetic acid. 22 g. of the resulting pyrazolone are dissolved in sodium hydroxide solution (5%), mixed with 7 g. of nitric and introduced with stirring into hydrochloric acid (10%), filtered with suction and the filtered substance dried. 12 g. of the isonitroso compound formed are reduced in the usual manner in 10 cc. of alcohol and 48 cc. of hydrochloric acid with 4.6 g. of tin sponge.

## EXAMPLE 12

1 - phenyl - 4 - amino - 5 - pyrazolone - 3 - carboxylic acid

|                                           |                 |
|-------------------------------------------|-----------------|
| g--                                       | 1.6             |
| Sodium sulfite anhydrous                  | g-- 45          |
| Hydroquinone                              | g-- 1.2         |
| Soda                                      | g-- 8           |
| Potassium-meta-bi-sulfite ( $K_2S_2O_5$ ) | g-- 4           |
| Potassium bromide                         | g-- 1           |
| Water                                     | cc-- Up to 1000 |

Normal negative developer; development periods: 10-12 minutes.

1 - phenyl - 4 - amino - 5 - pyrazolone - 3 - carboxylic acid is prepared as follows:

1 - phenyl - 5 - pyrazolone-3-carboxylic acid is reacted with benzene diazonium chloride as usual.

30.8 g. of the resulting azo dyestuff are suspended with 50 cc. of alcohol and

120 cc. of hydrochloric acid and then stirred with 25 g. of tin sponge until decolorization, filtered with suction, the filtered substance boiled with hydrochloric

acid (3%) and water, filtered with suction and the filtered substance washed with water.

What we claim is:

1. The process of developing silver halide layers which comprises applying to said layers a compound having a formula selected from the group consisting of



and



20 wherein  $R_1$  is a radical selected from the group consisting of  $-\text{OH}$ ,  $\text{O-alkyl}$ ,  $\text{O-aryl}$ ,  $\text{O-aralkyl}$ ,  $\text{NH}_2$ ,  $-\text{NH}-\text{NH}_2$ , and  $-\text{NH}-\text{OH}$ , and  $R_2$  is selected from the group consisting of hydrogen, alkyl, aralkyl, aryl and 2-tetrahydrothiophene sulfone radicals, in an alkaline medium.

2. A photographic developing composition consisting essentially of a compound having a formula selected from the group consisting of



and



30 wherein  $R_1$  is a radical selected from the group consisting of  $-\text{OH}$ ,  $\text{O-alkyl}$ ,  $\text{O-aryl}$ ,  $\text{O-aralkyl}$ ,  $\text{NH}_2$ ,  $-\text{NH}-\text{NH}_2$ , and  $-\text{NH}-\text{OH}$ , and  $R_2$  is selected from the group consisting of hydrogen, alkyl, aralkyl, aryl and 2-tetrahydrothiophene sulfone radicals, plus a compound selected from the group consisting of pyrocatechol, hydroquinone, pyrogallol, p-methyl-amino-phenol, N-p-oxyphenylglycin, and o- and p-phenylenediamines.

35 3. A photographic developer comprising a silver halide developing compound having a formula selected from the class consisting of:



and



40 wherein  $R_1$  is a radical selected from the group consisting of  $-\text{OH}$ ,  $\text{O-alkyl}$ ,  $\text{O-aryl}$ ,  $\text{O-aralkyl}$ ,  $\text{NH}_2$ ,  $-\text{NH}-\text{NH}_2$ , and  $-\text{NH}-\text{OH}$ , and  $R_2$  is selected from the group consisting of hydrogen, alkyl, aralkyl, aryl and 2-tetrahydrothiophene sulfone radicals, in an alkaline medium, together with a compound selected from the group consisting of pyrocatechol, hydroquinone, pyrogallol, p-methyl-amino-phenol, N-p-oxyphenylglycin, and ortho and para-phenylenediamines.

45 4. A photographic developer according to claim 3, wherein the first named compound is 1-phenyl-4-amino-5-pyrazolone-3-carboxylic acid amide.

5. A photographic developer according to claim 3, wherein the first named compound is 1-(p'-ethoxyphenyl)-4-amino-5-pyrazolone-3-carboxylic acid.

6. A photographic developer according to claim 3, wherein the first named compound is 4-amino-5-pyrazolone-3-carboxylic acid ethyl ester.

7. A photographic developer according to claim 3, wherein the first named compound is 1-phenyl-4-amino-5-pyrazolone-3-carboxylic acid hydrazide.

8. A photographic developer according to claim 3, wherein the first named compound is 1-(p'-aminophenyl)-4-amino-5-pyrazolone-3-carboxylic acid ethyl ester.

9. A photographic developer according to claim 3, wherein said silver halide developing agent is 1-phenyl-4-amino-5-pyrazolone-3-carboxylic acid.

10. In a silver halide developer mixture having a silver halide developer combined with an alkali metal sulfite, the improvement according to which the developer is a compound whose formula is selected from the group consisting of



wherein  $\text{R}_1$  is a radical selected from the group consisting of  $\text{OH}$ ,  $\text{O-alkyl}$ ,  $\text{O-aryl}$ ,  $\text{O-aralkyl}$ ,  $-\text{NH}_2$ ,  $-\text{NH}-\text{NH}_2$ , and  $-\text{NH}-\text{OH}$ , and  $\text{R}_2$  is selected from the group consisting of hydrogen, alkyl, aralkyl, aryl and 2-tetrahydrothiophene sulfone radicals.

11. The combination of claim 10 in which the silver halide developer is 1-phenyl-4-amino-5-pyrazolone-3-carboxylic acid amide.

#### References Cited in the file of this patent

##### UNITED STATES PATENTS

|           |                 |               |
|-----------|-----------------|---------------|
| 1,937,844 | Reed            | Dec. 5, 1933  |
| 2,139,870 | Wilmanns et al. | Dec. 13, 1938 |
| 2,637,732 | Schmid et al.   | May 5, 1953   |
| 2,731,473 | Taub            | Jan. 17, 1956 |

##### OTHER REFERENCES

- 25 Siewert: Chem. Abstracts, vol. 35, Col. 32 32 (1941).  
 Friedman: History of Color Photography, 1944, page 365.